

F. NIEMEYER.  
PROCESS OF LITHOGRAINING METAL PLATES.  
APPLICATION FILED FEB. 24, 1912.

1,045,068.

Patented Nov. 19, 1912.

FIG. 1.



FIG. 2.



FIG. 5.



FIG. 3.



FIG. 4.



Witnesses:

A. B. Mattingly

J. D. Penney

Inventor:

Frederick Niemeyer.

By his Attorney, F. H. Richards,

# UNITED STATES PATENT OFFICE.

FREDERICK NIEMEYER, OF HOBOKEN, NEW JERSEY.

## PROCESS OF LITHOGRAINING METAL PLATES.

1,045,068.

Specification of Letters Patent. Patented Nov. 19, 1912.

Application filed February 24, 1912. Serial No. 370,745.

To all whom it may concern:

Be it known that I, FREDERICK NIEMEYER, a citizen of the United States, residing in Hoboken, in the county of Hudson and State of New Jersey, have invented certain new and useful Improvements in Processes of Lithograining Metal Plates; of which the following is a specification.

This invention relates to the manufacture of surface-grained metal plates for use in the art of printing by the lithographic method.

The object of my present invention is to produce on a metal plate, especially on plates of zinc, a finely-grained surface in which the elevations or "grain" shall be or consist of the solid metal free of coating substances or adherent salts, and shall be of a character to take and properly hold the substance, while resisting the force, of the artist's pencil when the plate is being prepared for use by such method, and also to receive the figures or outlines when applied thereto by the usual transfer method; and, to furnish such a grained plate which shall have its interstices, or the spaces between such elevations, of a depth and character proper and effective for taking and holding the required amount of water, or moisture, in the areas between the treated or ink-holding areas, while the plate is in use on a lithographic printing-press.

In the accompanying drawing illustrative of my present improvements in lithographic printing plates.—Figure 1 is a sectional side view of a receptacle with a plate therein for treatment while submerged in a bath of the character hereinafter described. Fig. 2 is a similar view showing the receptacle in a changed position, it being tilted toward the left-hand, and adapted to be also reversely tilted toward the right-hand, whereby to subject the surface of the plate to a relatively forcible washing action. Fig. 3 is a fragmentary and diagrammatic view, similar to a portion of Fig. 1 but greatly enlarged, for illustrating the following description regarding the deposition of granules by flotation and gravity. Fig. 4 is a view similar to Fig. 3 but much more enlarged, for illustrating certain portions of the following description and explanations; and Fig. 5 is a view supplemental to Fig. 4.

Similar characters designate like parts in all the views.

In preparing to treat a plate by my process, I place the plate, as P, in some suitable receptacle, as C, of a depth to hold the bath E, when the receptacle is standing level, as in Fig. 1, and also when tilted, as in Fig. 2. 60 The size and proportions of the receptacle should, of course, be suitable for the size of plate to be treated, and for using a sufficient quantity of the fluid bath of the required character. When the quantity of the fluid is 65 larger, of course it will not need to be renewed so often; but I prefer to keep the bath effective by using only a moderate quantity and then renewing with sufficient frequency. 70

For the bath E, water acidulated with some suitable acid may be used, and for treating zinc I preferably employ nitric acid for that purpose, but only of a strength to act rather slowly upon the metal surface. 75 In practice I usually employ about one part of the ordinary fluid acid of commerce to about fifty parts of water, but this may be varied in order to regulate the rapidity of reduction of the metal surface. 80

As a means for regulating or properly modifying the distribution and the regularity of the metal-reducing action, to form the desired inequalities of surface and so produce the grain, I add to the bath a quantity of sedimentation material in the form of granules or fine particles adapted to be readily brought to flotation and having an acid-resistant quality, and having such a specific gravity as to settle or deposit on the plate 90 in a slow and progressive manner, so that the granules accumulate on the plate in a constantly increasing layer or depth during the action of the acid on said plate. Thus the plate is concurrently subjected to reduction by the acid and to a modifier consisting of a deposition or sedimentation of a flotation material accumulating thereon during the action of the acid. In practice, I prefer granules having a specific gravity of between one and one-half and two and one-half times that of water, depending somewhat on the fineness and shapes of the granules, and somewhat, also, on the acidity of the bath. 95 100 105 110

The flotation of the granules is indicated at P' Figs. 1 and 2, where the small granules are for the time being in suspension or flotation; and in practice many of them so remain, practically continuously, but this 110

has, I find, slight if any disadvantage. On the bath E standing still for even a brief time, many of the granules f become deposited by gravity into a relatively evenly spread layer upon the plate-surface S, approximately as indicated for instance at g, Figs. 3 and 4; and, by reason, as I suppose, of the chemical and voltaic or other qualities of the materials, and of the conditions thus established, the surface S is at once subjected to a reducing action of such a character as to tend to form a grain therein of the quality and water-retaining capacity required in the lithographic art.

When the plate is in the acidulated bath and at a suitable distance below the surface thereof, the granules continue accumulating on the plate while the acid is eating away the surface of the metal. The greater the depth of the bath over the plate, the greater will be the amount of that accumulation, or deposition during a given time and from a given initial proportion or quantity of the granules in the fluid. Therefore by suitably regulating those proportionate amounts and the depth of the fluid, the rapidity of the granule-deposition may be controlled within proper limits, which in practice are ascertainable by trial and observation of the amounts of surface reduction in given times, for the production of such a coarseness and depth of the grain as may be desired.

When the reducing action proceeds for a short time certain dissociations appear to take place, with the formation of salts which by their position on the plate-surface tend to reduce and suspend the chemical or metal-reducing action, and therefore I subject the plate at intervals to a washing or clearing operation which may be performed by flowing the bath over the surface with sufficient force for thereby dislodging such accumulations or deposits,—if any there may be produced,—and then again cover the plate by the deposition of the granules thereon by gravity, when the reduction process goes on again; these successive steps or stages are repeated to the extent required for bringing the grain up to the desired depth and formation. At each successive re-deposition of the granules, the undulations then already produced tend to modify, as I apprehend, the manner of such new deposition, so that the metal is removed by successive stages in which any particular small area, or given area,—such for instance as one of a size less than that of a granule,—is deepened little by little, while at each successive stage such obstructive salts as may have been formed on the surface, S, are cleared off by the washing operation.

The acid begins acting upon the metal over nearly the whole surface, and it appears to be probable that the metal-reducing action is in some way progressively modified as to the distribution of the points of relatively greater and lesser effect, during the progress of the deposition which accumulates upon the plate. When by the agitation of the bath, however performed, the flotation of the granules is accomplished, the acid will, of course, act about equally over the entire surface of the metal, and will, as I suppose, become variable or irregular during the immediately subsequent and gradual re-deposition by gravity of the flotation material. By repeating the flotation at frequent intervals while continuing the plate in the bath, the metal is subjected to successive treatments which in one respect are each of a similarly varying or progressive character, since during each said treatment the restriction of the metal-reducing action goes on progressively from a beginning at which this action extends over the whole, or nearly the whole, surface and is thereafter progressively reduced toward or nearly to the point of cessation.

In practice it will usually be sufficient to carry this progressive reduction only to a point where there is a substantial lessening of the metal-reducing action, and then clear off the accumulation on the plate of the flotation-material and also at the same time clear off such products as may have been formed by the action of the acid-bath and the metal removed thereby from the plate. This step being performed, including the re-flotation of the granular material, the re-deposition again begins and goes on as before, for subjecting the partially grained surface to a further stage of reduction; and so on, until the depth and character of grain is obtained, as may be required.

When the surface S has been reduced to a partially-formed grain, and the surface is cleared of such obstructive salts, aqueous or otherwise, as may have been formed between the metal of the plate and a metal of the granules, it is evident that on a re-deposition on the plate of the said granules, these will normally deposit or form the lower series or layer, g, Fig. 5, in an undulating arrangement or formation, so that the specific relations of those metal elements to the grain of the plate will naturally be modified at each successive re-deposition stage of the process. This feature will be understood by comparing Figs. 4 and 5, in view of the preceding explanations. The plate P with its partially grained surface S' is shown with granules, g'', re-deposited thereon in an undulating and irregular arrangement, such as naturally would be caused by the process above set forth, when the granules fall by a slow and gentle action through a fluid upon an undulating surface. Each successive stage of the process, therefore, is not merely a repetition of the first, or of a next preceding stage.

ing stage, but may properly be considered as differing from the next preceding stage, since each successive re-deposition is made on a more advanced formation of the grain-  
5 surface of the plate.

As a suitable flotation-material, I prefer-  
ably employ some metallic salt which is not  
materially reduced or affected by the acid-  
bath, when this is of the moderate degree of  
10 strength or acidity which is sufficient for  
slowly eating away the metal surface; and  
which, at the same time has a granular form,  
preferably of a flake-like character, and has  
the granules of a size suitable for the fine-  
15 ness of grain desired, and of a specific grav-  
ity low enough to prevent a too rapid accum-  
ulation on the plate after any re-flotation  
of this material in the bath.

One kind of granule or flotation material  
20 which I employ, more especially for treat-  
ing zinc plates, is a compound material com-  
pounded preferably of the salts of two  
metals, and preferably of two metals other  
25 than zinc; and other than the metal of the  
plate, when this is not of zinc. One such  
material is a compound formed from iron  
and copper which, because of its resist-  
ance to the acid of the bath and the small  
30 size and low weight of its granules, pro-  
duces by flotation and gravity a deposi-  
tion of good quality and effect. For this  
compound I prefer one of the formulas  
 $FeCy + 2CuCy$ . This material appears to  
35 be particularly suitable because of the  
qualities above mentioned, and also, as I  
apprehend, because of its effect on, or the  
part it takes in certain reactions, which it  
appears may take place during or incident  
40 to the metal-reducing action upon the plate  
while in the bath.

While I am unable and deem it unneces-  
sary at this time to fully set forth and ex-  
plain the specific phenomena which evi-  
dently or probably occur in the solution,  
45 such for instance as the ionization and the  
voltaic action, or such others as may take  
place, I apprehend that in some manner the  
granules of the copper and iron salts operate  
50 to modify the chemical and electrolytic  
actions and reactions upon the zinc and to  
relatively localize or accentuate the metal-  
reducing action upon a great number of  
minute areas, and thus regulate or control  
55 the reduction of the plate-surface to the de-  
sired grain-formation; and, I apprehend this  
may be due to some intimate connection be-  
tween chemical activity and electrical con-  
ductivity, since the acid, especially nitric  
60 acid, employed as the electrolytic element,  
appears to have the proper, and a relatively  
high, electrical conductivity. One explana-  
tion as to the way these reducing actions  
may perhaps be regulated, I have indicated  
65 in Fig. 3, where a layer of the metal-salt  
granules,  $g$ , lie close to the surface  $S$ , while

other granules, as  $g'$ , are more or less super-  
posed on such first layer. As a result, there  
are formed great numbers of minute inter-  
vening spaces, as  $t$ , Figs. 4 and 5, between  
70 compounds of metals which have the rela-  
tive character of electrodes, while these  
spaces are filled with a fluid having the  
character of an electrolyte, thereby produc-  
ing, as I suppose, some kind and degree of  
75 voltaic relationship or condition whereby  
the usual and corresponding changes are  
effected in the several metals or elements by  
reactions involving the electrolytic element.  
Not only are the electrically different metals  
80 connected by the same electrolyte, but the  
resultant chemical action may produce a  
difference in the strength of this electrolyte  
in the spaces  $t$ , and so in some manner cause  
an unequal amount and distribution of such  
85 chemical action on the surface  $S$ .

When a granule falls or is deposited on  
the plate-surface, it acts in a mechanical  
way to displace the fluid at that point, and  
this normally tends, I understand, to re-  
strict or reduce the action of the acid in  
90 the minute area so covered by the granule,  
which may be said to form an obstacle at  
such point against the free approach of  
the acid to that area. Thus the granules  
may be said to operate in several respects  
95 or capacities, especially when formed of a  
double salt, and still more so, when formed  
of a double cyanate,—first, mechanically;  
second, chemically, and also most probably,  
by catalysis, including the phenomena in-  
100 volved in the electro-osmotic relations of the  
substances in the granules, the bath and the  
plate.

The acid resistant granules may be com-  
posed of some suitable single substance, but  
105 I prefer in practice, to use granules com-  
posed of one of that class of compounds or  
salts which are sometimes designated as  
double-salts, and of these I preferably em-  
ploy a double-salt of two different metals,  
110 and to have each of these different from the  
metal of the plate which is to be grained.  
Thus for treating zinc, I preferably employ  
salts of iron and copper, each different from  
zinc; and of these compounds or salts I  
115 preferably employ the iron-cyanogen and  
copper cyanogen salts, respectively, and of  
these I prefer to employ the cyanates, and  
to have the copper-salt or cyanate in excess  
of the iron salt or cyanate. Although zinc  
120 is classed as a divalent metal, it appears in  
some cases to be able in reactions involving  
a plurality of other metals, to replace some  
other divalent metals, including iron; and,  
perhaps, copper, which is classed as both  
125 monovalent and divalent. In such reactions  
so far as occurring in my process, I ap-  
prehend that some of the phenomena of  
catalysis may also occur. Also, it may be  
noted that as regards the osmotic action or  
130

pressure or the electro-osmotic value in solutions, iron is classed as having a negative electro-motive force, whereas, in comparison, both zinc and copper are classed as 5 having a positive electrolytic, or electro-osmotic quality or value. Thus in treating zinc plates with a flotation-material having a salt of iron and a salt of a more positive metal, (such as copper for instance), the 10 granules are composed in part of the salt of a metal which is, as regards its electro-osmotic character, negative relatively to the zinc and also relatively to the metal of the other salt of the compound of which the 15 granules are formed.

When the gravitating granules are composed of a compound of cyanogen salts of iron and copper, and when the iron-cyanogen salt is a cyanate, that compound will 20 therefore comprise two metal-cyanogen salts of which one is the cyanate of a divalent metal (iron) having an electro-osmotic value relatively negative to the zinc and also to the metal (copper) of the other metal- 25 cyanogen salt. Owing to their low specific gravity and their size and character, this kind of granules are readily floatable by agitation of the bath, and are deposited therefrom onto the plate surface in a slow and 30 regular manner particularly favorable for the requirements of this method of making the litho-grain.

In this process, the object is to reduce the original plane surface to a grain-surface, 35 rather than to supply such a grain as an addition to the plate. In view of this purpose, and also for convenience, I designate the process as one for litho-graining metal-plates, thus referring to the adaptability 40 of the plates when so grained for use in the art of lithographic printing.

While a granule of the double cyanate rests on the zinc surface, the molecule of iron-cyanate may be considered as being 45 held in place by its association with the molecule of copper-cyanate, and thus may part with some of its cyanogen directly to the zinc, which has a strong affinity therefore; and such an exchange may, I infer, be 50 aided by the oxygen supplied by the nitric acid to the iron, as well as, in part, to the zinc; and, owing to the minuteness of the granule, that exchange or reaction may therefore take place, as to each such granule 55 only in a correspondingly minute area, with the result of forming a great number of closely arranged but distinct points of reduction on the zinc surface.

When a sufficiently dilute acid bath is 60 used, the metal-plates, particularly zinc plates, may be subjected to a primary reduction which is initially distributed over the whole surface and is then gradually restricted both as to the distribution and the

regularity of the reduction, this being accomplished by a progressive gravitational deposition of an acid-resistant flotation-material; and, next, subjected to a second reduction by repeating the said operation on the primarily-reduced plate-surface; and 70 then subjected to a further reduction by repetitions of the said operation on the secondarily-reduced plate surface, whereby the final surface is obtained by three or more successive reductions, each of which begins 75 with the plate-surface at a different stage of grain-formation.

In litho-graining metal-plates in the foregoing manner, the grain is developed or produced in a clean and effective condition, being formed or composed of the solid metal and free of adherent films, deposits or coatings, and without the formation of substantial salts or the like to impair the quality of the surface-grain for use in lithographic 85 printing. On zinc plates, the process may be properly carried out in from three to eight minutes, depending on the strength of the acid, the depth of the bath over the plate, the quantity of the flotation-material in the 90 bath, and the frequency of the re-flotation and re-deposition of the granules of that material. In practice I prefer to so regulate those periods and quantities as to provide for from three to six of the said 95 depositions during the complete operation.

In applying my present process to the graining of plates of metals other than zinc, such an aluminum or copper, either pure or alloyed, other dilute acids, instead of the 100 nitric acid, may be used, preferably selecting such a kind and degree of dilution of the acid as will act slowly on the metal-surface, and thus give time for the desired number of re-depositions of the flotation material 105 during the process. In some instances such other acids may be used in graining the zinc plates, especially when the compounds or salts, whether cyanates or not, of which the granules are composed, shall be of a character to work in harmony with the particular kind of acid employed and not be rapidly consumed or neutralized in the bath.

Having thus described my invention, I 115 claim:

1. The process of litho-graining metal-plates, which consists in reducing the plate-surface in an acid bath under an accumulating deposition by gravity of granules which are floatable by agitation of the bath 120 and are resistant to the acid.

2. The process of litho-graining metal-plates, which consists in reducing the plate-surface in an acid bath under an accumulating deposition from flotation of granules 125 and continuing such reduction to the point of forming a partial grain, next clearing off the plate-surface and refloating the granules,

- and then subjecting the plate-surface to further reduction under an accumulating re-deposition of the granules. 70
8. That improvement in the art of litho-graining metal-plates, which consists in subjecting the plate-surface in an acid bath to a primary reduction initially distributed over the whole surface and then gradually restricting that distribution and the regularity of that reduction by the gravitational deposition of an acid-resistant flotation-material, and next subjecting the surface to an additional reduction by repeating the said operations on the plate surface after such primary reduction. 75
9. That improvement in the art of litho-graining metal-plates, which consists in subjecting the plate-surface in an acid bath to a primary reduction initially distributed over the whole surface and then gradually restricting that distribution and the regularity of that reduction by the gravitational deposition of an acid-resistant granular flotation-material, and next subjecting the surface to successive additional reductions after such primary reduction, by subjecting the plate-surface to repeated gravitational depositions of the flotation granules while continuing the acid treatment. 80
10. The process of litho-graining metal-plates, which consists in reducing the plate-surface in an acid bath containing in flotation gravitating granules of a double salt of two different metals, and continuing the acid treatment while accumulating a gravitational deposition of such flotation material upon the plate-surface. 85
11. The process of litho-graining metal-plates, which consists in reducing the plate-surface in an acid bath containing in flotation gravitating granules of a double salt of iron and copper, and continuing the acid treatment while accumulating a gravitational deposition of such flotation material upon the plate-surface. 90
12. The process of litho-graining metal-plates, which consists in reducing the plate-surface in an acid bath containing in flotation gravitating granules of a double salt of iron and copper, and containing the acid treatment during successive gravitational re-depositions of such flotation material. 95
13. The process of litho-graining metal-plates, which consist in reducing the plate-surface in an acid bath containing in flotation gravitating granules of a double salt of iron and copper and having the copper-salt in excess of the iron-salt, and continuing the acid treatment while accumulating a gravitational deposition of such flotation material upon the plate-surface. 100
14. The process of litho-graining metal-plates, which consists in reducing the plate-surface in an acid bath containing in flotation gravitating granules of a double salt of iron and copper and having the copper-salt in excess of the iron-salt, and continuing the acid treatment during successive gravitational re-depositions of such flotation material. 105
15. The process of litho-graining metal-plates, which consists in reducing the plate-surface in an acid bath containing in flotation gravitating granules composed of the cyanates of two different metals, and continuing the acid treatment while accumulating a gravitational deposition of such flotation material upon the plate-surface. 110
16. The process of litho-graining metal-plates, which consists in reducing the plate-surface in an acid bath containing in flotation gravitating granules composed of the cyanates of two different metals, and continuing the acid treatment during successive gravitational re-depositions of such flotation material. 115
17. The process of litho-graining metal-plates, which consists in reducing the plate-surface in an acid bath containing in flotation gravitating granules composed of the cyanates of two different metals, and containing the acid treatment during successive gravitational re-depositions of such flotation material. 120
18. The process of litho-graining metal-plates, which consists in reducing the plate-surface in an acid bath containing in flotation gravitating granules composed of the cyanates of two different metals, and containing the acid treatment during successive gravitational re-depositions of such flotation material. 125
19. The process of litho-graining metal-plates, which consists in reducing the plate-surface in an acid bath containing in flotation gravitating granules composed of the cyanates of two different metals, and continuing the acid treatment during successive gravitational re-depositions of such flotation material. 130

plates, which consists in reducing the plate-surface in an acid bath containing in flotation gravitating granules composed of the cyanates of two different metals other than the metal of the plate, and continuing the acid treatment while accumulating a gravitational deposition of such flotation material upon the plate-surface.

18. The process of litho-graining metal-  
10 plates, which consists in reducing the plate-  
surface in an acid bath containing in flota-  
tion gravitating granules composed of the  
cyanates of two different metals other than  
the metal of the plate, and continuing the  
acid treatment during successive gravi-  
15 tational re-depositions of such flotation ma-  
terial.

19. The process of litho-graining metal-  
20 plates, which consists in reducing the plate-  
surface in an acid bath containing in flota-  
tion gravitating granules composed of a  
compound metallic salt comprising an iron-  
cyanogen salt, and continuing the acid treat-  
25 ment during a gravitational deposition of  
such flotation material upon the plate-surface.

20. The process of litho-graining metal-  
20 plates, which consists in reducing the plate-  
surface in an acid bath containing in flota-  
tion granules composed of a compound  
metallic salt comprising an iron-cyanogen  
salt, and continuing the acid treatment dur-  
ing successive re-depositions by gravity of  
such flotation material.

21. The process of litho-graining metal-  
35 plates, which consists in reducing the plate-  
surface in an acid bath containing in flota-  
tion gravitating granules composed of the  
cyanates of two different metals other than  
the metal of the plate and one of which  
40 is iron, and continuing the acid treatment  
while accumulating a gravitational deposi-  
tion of such flotation material upon the  
plate-surface.

22. The process of litho-graining metal-  
45 plates, which consists in reducing the plate-  
surface in an acid bath containing in flota-  
tion gravitating granules composed of the  
cyanates of two different metals other than  
the metal of the plate and one of which is  
50 iron, and continuing the acid treatment dur-  
ing successive gravitational re-depositions  
of such flotation material.

23. The process of litho-graining metal-  
55 plates, which consists in reducing the plate-  
surface in an acid bath containing in flota-  
tion gravitating granules composed of the  
cyanates of iron and copper, and continuing  
the acid treatment while accumulating a  
60 gravitational deposition of such flotation  
material upon the plate-surface.

24. The process of litho-graining metal-  
65 plates, which consists in reducing the plate-  
surface in an acid bath containing in flota-  
tion gravitating granules composed of the

cyanates of iron and copper, and continuing  
the acid treatment during successive  
gravitational re-depositions of such flota-  
tion material.

25. The process of litho-graining metal-  
70 plates, which consists in reducing the plate-  
surface in an acid bath containing in flota-  
tion gravitating granules composed of the  
cyanates of iron and copper and having the  
copper-cyanate in excess of the iron-cya-  
75 nate, and continuing the acid treatment  
while accumulating a gravitational depo-  
sition of such flotation material upon the  
plate-surface.

26. The process of litho-graining metal-  
80 plates, which consists in reducing the plate-  
surface in an acid bath containing in flota-  
tion gravitating granules composed of the  
cyanates of iron and copper and having the  
copper-cyanate in excess of the iron-cya-  
85 nate, and continuing the acid treatment  
during successive gravitational re-deposi-  
tions of such flotation material.

27. The process of litho-graining metal-  
90 plates of zinc, which consists in reducing  
the plate-surface in an acid bath containing  
in flotation gravitating granules composed  
of salts of two metals other than the metal  
95 of the plate and one of which is iron, and  
continuing the acid treatment while accu-  
mulating a gravitational deposition of such  
flotation material upon the plate-surface.

28. The process of litho-graining metal-  
100 plates of zinc, which consists in reducing  
the plate-surface in an acid bath containing  
in flotation gravitating granules composed  
of salts of two metals other than the metal  
105 of the plate and one of which is iron, and  
continuing the acid treatment during suc-  
cessive re-depositions of such flotation ma-  
terial.

29. The process of litho-graining metal-  
110 plates of zinc, which consists in reducing  
the plate-surface in an acid bath containing  
in flotation gravitating granules composed  
of cyanates of two metals other than the  
metal of the plate and one of which is iron,  
115 and continuing the acid treatment while ac-  
cumulating a gravitational deposition of  
such flotation material upon the plate-sur-  
face.

30. The herein described process of litho-  
120 graining metal-plates of zinc, which con-  
sists in reducing the plate-surface in an acid  
bath containing in flotation gravitating  
granules composed of cyanate of two met-  
als other than the metal of the plate and  
125 one of which is iron, and containing the  
acid treatment during successive gravi-  
tational re-depositions of such flotation mate-  
rial.

31. The process of litho-graining metal-  
130 plates of zinc, which consists in reducing  
the plate-surface in an acid bath containing  
in flotation gravitating granules composed

of salts of iron and copper, and continuing the acid treatment while accumulating a gravitational deposition of such flotation material upon the plate-surface.

5 32. The process of litho-graining metal-  
plates of zinc, which consists in reducing the plate-surface in a dilute nitric acid bath containing in flotation gravitating granules composed of salts of iron and copper, and  
10 continuing the acid treatment during suc-  
cessive gravitational re-depositions of such flotation material.

33. The process of litho-graining metal-  
plates of zinc, which consists in reducing the plate-surface in an acid bath containing in flotation gravitating granules composed of a compound salt which comprises an iron-cyanogen salt, and continuing the acid treatment while accumulating a gravitational deposition of such flotation material upon the plate-surface.

34. The process of litho-graining metal-  
plates of zinc, which consists in reducing the plate-surface in an acid bath containing in flotation gravitating granules composed of a compound salt which comprises an iron-cyanogen salt and a copper-cyanogen salt, and continuing the acid treatment during successive re-depositions of such flotation material.

35. The process of litho-graining metal-  
plates of zinc, which consists in reducing the plate-surface in an acid bath containing in flotation gravitating granules composed of a plurality of salts which comprise at least one cyanate of a metal, and continuing the acid treatment during a gravitational deposition of such flotation material upon the plate-surface.

40 36. The herein described process of litho-  
graining metal-plates of zinc, which con-  
sists in reducing the plate-surface in an acid bath containing in flotation granules com-  
posed of a plurality of salts which com-  
prises at least one cyanate of a metal, and  
continuing the acid treatment during suc-  
cessive re-depositions of such flotation ma-  
terial.

37. The process of litho-graining metal-  
plates of zinc, which consists in initially re-  
ducing the plate-surface in a dilute nitric acid bath containing in flotation gravitating granules composed of a compound me-  
talic salt which comprises an iron-cyanogen salt and a copper-cyanogen salt and having one of these salts a cyanate, and then further forming the grain by continu-  
ing the acid treatment during successive re-depositions of such flotation material.

60 38. The process of litho-graining plates of divalent metal having a positive electro-  
osmotic value, which consists in reducing the plate-surface in an acid bath containing in flotation gravitating granules composed of salts of two different metals of which

one is a divalent metal having in the acid bath a relatively negative electro-osmotic value, and containing the acid treatment while progressively accumulating a gravitational deposition of such flotation mate-  
rial upon the plate-surface.

39. The process of litho-graining plates of divalent metal having a positive electro-  
osmotic value, which consists in reducing the plate-surface in an acid bath containing in flotation gravitating granules composed of salts of two different metals of which one is a divalent metal having in the acid bath a relatively negative electro-osmotic value, and continuing the acid treatment during successive gravitational re-depositions of such flotation material upon the plate-surface.

40. The process of litho-graining metal-  
plates of zinc, which consists in reducing the plate-surface in an acid bath containing in flotation gravitating granules composed of a compound of metallic salts which comprises two metal-cyanogen salts of which one is the cyanate of a divalent metal having an electro-osmotic value relatively negative in the bath to the zinc and also the metal of the other metal-cyanogen salt, and continuing the acid treatment while progressively accumulating a gravitational deposition of such flotation material upon the plate-surface.

41. The process of litho-graining zinc metal-plates of zinc, which consists in reduc-  
ing the plate surface in an acid bath con-  
taining in flotation gravitating granules composed of a compound of metallic salts which comprises two metal-cyanogen salts of which one is the cyanate of a divalent metal having an electro-osmotic value relatively negative in the bath to the zinc and also to the metal of the other metal-cyanogen salt, and continuing the acid treatment during successive gravitational re-deposi-  
tions of such flotation material.

42. The process of litho-graining metal-  
plates of zinc, which consists in reducing the plate-surface in an acid bath containing in flotation gravitating granules composed of a substance which comprises the cyanate of a metal having an electro-osmotic value which is negative relatively to the zinc, and continuing the acid treatment while accumulating a deposition of such flotation material upon the plate-surface.

43. The process of litho-graining metal-  
plates of zinc, which consists in reducing the plate-surface in an acid bath containing in flotation gravitating granules composed of a substance which comprises the cyanate of a metal having an electro-osmotic value which is negative relatively to the zinc, and continuing the acid treatment during successive re-depositions of such flotation ma-  
terial upon the plate-surface.

44. The herein described process of litho-graining metal-plates of zinc, which consists in reducing the plate-surface in an acid bath containing in flotation granules composed of a compound of metallic salts, which comprises the cyanates of two metals other than zinc and having, respectively, relatively negative and positive electro-osmotic values, and one of these having its 5 said value negative relatively to that of the zinc, and continuing the acid treatment while accumulating a gravitational deposition of such flotation material upon the plate-surface.
45. The process of litho-graining metal-plates of zinc, which consists in reducing the plate-surface in an acid bath containing in flotation granules composed of a compound of metallic salts, which comprises the 10 cyanates of two metals other than zinc and having, respectively, relatively negative and positive electro-osmotic values, and one of these having its said value negative relatively to that of the zinc, and continuing 15 the acid treatment during successive redepositions of such flotation material upon the plate-surface.
46. That improvement in the art of litho-graining metal-plates of zinc, which consists in subjecting the plate-surface in an acid bath to a primary reduction initially distributed over the whole surface and then gradually restricting that distribution and the regularity of that reduction by a progressive gravitational deposition of an acid- 20
- resistant flotation-material; next subjecting the surface to a second reduction by repeating the said operation on the primarily-reduced plate-surface; and then subjecting the surface to a third reduction by again 25 repeating the said operation on the secondarily-reduced plate-surface, whereby the final surface is obtained by three successive reductions, each of which begins with the plate-surface at a different stage of grain-formation. 30
47. That improvement in the art of litho-graining metal-plates of zinc, which consists in subjecting the plate surface in an acid bath to a primary reduction initially 35 distributed over the whole surface and then gradually restricting that distribution and the regularity of that reduction by a progressive gravitational deposition of an acid-resistant flotation-material; next subjecting the surface to a second reduction by repeating the said operation on the primarily-reduced plate-surface; and then subjecting the surface to a plurality of further reductions by successively repeating the said operation on the partially-reduced plate surface, whereby the final surface is obtained by at least four successive reductions, each 40 of which begins with the plate-surface at a different stage of grain-formation. 45
48. That improvement in the art of litho-graining metal-plates of zinc, which consists in subjecting the plate-surface in an acid bath to a primary reduction initially 50 distributed over the whole surface and then gradually restricting that distribution and the regularity of that reduction by a progressive gravitational deposition of an acid-resistant flotation-material; next subjecting the surface to a second reduction by repeating the said operation on the primarily-reduced plate-surface; and then subjecting the surface to a plurality of further reductions by successively repeating the said operation on the partially-reduced plate surface, whereby the final surface is obtained by at least four successive reductions, each 55 of which begins with the plate-surface at a different stage of grain-formation. 60

FREDERICK NIEMEYER.

Witnesses:

H. D. PENNEY,  
JOHN MORRIS.